

April 29, 1958

R. KUNIN

2,832,727

ELECTROLYTIC PRECIPITATION OF URANIUM  
FROM THE ION EXCHANGE ELUATES  
Filed April 7, 1954



INVENTOR.  
ROBERT KUNIN

BY *John F. Bergin*  
ATTORNEY

## ELECTROLYTIC PRECIPITATION OF URANIUM FROM THE ION EXCHANGE ELUATES

Robert Kunin, Trenton, N. J., assignor, by mesne assignments, to the United States of America as represented by the United States Atomic Energy Commission

Application April 7, 1954, Serial No. 421,667

11 Claims. (Cl. 204—1.5)

This invention relates to the recovery of uranium. It relates to an electrolytic process wherein uranium oxide and/or hydroxide is precipitated and is isolated from aqueous solutions which contain soluble uranium salts.

In the leaching of uranium-bearing ores the uranium is extracted as a complex anion of an acid. In a subsequent step, the solution of the complex acid is passed through a column or bed of particles of an ion exchange resin, preferably a strongly basic, quaternary ammonium, anion exchange resin. The uranium complex is adsorbed by the anion exchange resin and is removed from the leach liquor. Next, an aqueous solution of a mineral acid and an alkali metal or ammonium salt of the mineral acid, such as a solution of nitric acid and sodium nitrate, is passed through the mass of resin. The uranium is thereby removed; i. e., eluted, in the form of a dissolved uranyl salt having the formula  $UO_2(X)_2$  in which X is one equivalent weight of an acid radical such as a nitrate radical,  $—NO_3$ , sulfate radical,  $—SO_4$ , or a chloride radical,  $—Cl$ . This solution of uranyl salt which also contains some of the acid and salt is called the eluate.

The object of this invention is to treat such an eluate so as to convert the uranyl salt into the form of an insoluble hydrated oxide which can be readily isolated and ignited to the oxide,  $U_3O_8$ .

This object is accomplished efficiently and economically by a method of electrolysis wherein a direct electric current is passed through an electrolytic cell which is divided by means of a permselective membrane into a cathode compartment containing the above-mentioned eluate and an anode compartment containing a solution of an alkali metal salt or an ammonium salt—preferably a sodium salt—of the acid which was used for elution. Preferably the anolyte is a solution of sodium nitrate or sodium chloride.

The electrolytic cell which is employed can best be understood by a reference to the attached drawing wherein in the single figure is a diagrammatical representation of a typical cell which is divided into an anode compartment and a cathode compartment by means of a permselective membrane or diaphragm. In said figure, 1 represents a container which is divided into two compartments, 5 and 6, by a permselective membrane, 2, which is described in greater detail below. Compartment 5 is an anode compartment by virtue of the presence there of the anode 3, while compartment 6 is a cathode compartment because it contains the cathode 4. When the cell is in operation, the electrodes are connected to a source of electric power not shown.

The cell which is employed in this invention can be varied as to size, shape, vents, ports, exits, construction materials, controls, embellishments, et cetera without departing from the spirit of this invention. What is essential is that the cell have two compartments, one containing the anode and the other containing the cathode, and that the two compartments be separated by a permselective membrane as defined herein.

The permselective membranes which divide the electrolysis cell into the two compartments are all important to the success of this process. They function by allowing only ions of one sign—either anions or cations—to pass through them while at the same time preventing the passage of ions of the opposite sign from one compartment to the other. Cationic permselective membranes are those which allow the passage of cations while anionic permselective membranes are those which permit the passage of anions. The membranes contain ion exchange resins and it is the presence of the ion exchange resins which imparts the property of permselectivity. While the composition of the permselective membranes can vary within reasonable limits, it is important that they contain enough ion exchange resin as to have suitably high conductance when employed in the electrolysis cell. The permselective films which have proven to be most suitable for use in this process are those made by incorporating particles of an ion exchange resin in a film-forming matrix such as polyethylene or vinyl resins. Such membranes are available commercially.

In the process of this invention, an eluate which is an aqueous solution of a uranyl salt together with a mineral acid and an alkali metal salt or an ammonium salt of the mineral acid is placed in the cathode compartment of the electrolysis cell. The anolyte which is employed is ordinarily a solution of the same alkali metal salt or ammonium salt as is present in the eluate.

As electrolysis proceeds, hydrogen is liberated at the cathode, the catholyte decreases in acidity, and the  $UO_2^{++}$  ion is reduced to  $U^{+++}$ . The uranium commences to precipitate as an oxide and continues to do so as the pH of the catholyte gradually approaches neutral. As neutrality is reached, the precipitation is essentially complete, and the electrolysis could be terminated. It has been noticed that if the electrolysis is continued for just a few seconds the pH of the catholyte will rise almost perpendicularly, if charted graphically, from the neutral point to as high as 12. This fact makes it very simple to determine the end of the electrolysis and is a handy analytical or process control tool. However, it should be noted that electrolysis is carried out, for all intents and purposes, with an acidic catholyte.

The precipitate is readily removed from the catholyte by conventional means such as filtration or centrifuging and is ultimately ignited to  $U_3O_8$ . At the same time, when an anionic permselective membrane is employed, anions such as sulfate, nitrate or chloride ions migrate from the cathode compartment through the anionic membrane into the anode compartment. When chloride ions are involved, some chlorine is liberated at the anode. When nitrate or sulfate ions are involved, there is a liberation of oxygen. In any case, however, the anolyte becomes increasingly acidic and ultimately reaches the point where it contains both salt and acid. At this point it is entirely suitable for eluting more adsorbed uranium complex from another bed of exhausted anion-exchange resin. During electrolysis, cations in the anolyte migrate toward the cathode but are constrained from entering the cathode compartment by the anionic membrane which, because it is anionic, allows the passage of only anions.

When a cationic permselective membrane is employed, alkali metal ions in the anolyte migrate through the membrane into the catholyte and the current is carried by them. In such a case, however, the ultimate result is the same as when an anionic membrane is used. Uranium is precipitated in the cathode compartment and the anolyte becomes acidic so that it can be used for elution. Furthermore, after removal of the uranium, the catholyte contains alkali metal salts and it can be, and should be, used as the anolyte in the electrolysis of subsequent batches of eluate.

Actually, the electrolytic process described above can be combined with the operation of beds of anion-adsorbing resins in a cyclic or continuous process. For example, an eluate is run into the cathode compartment of the electrolytic cell described above through which is passing a direct current. As the uranium precipitates, the catholyte is removed and filtered and the filtrate is passed into the anode compartment. At the same time the anolyte which has become acidic is withdrawn and is used for eluting a bed of anion exchange resin which contains adsorbed uranium complex.

It is, therefore, apparent that by means of this electrolytic process uranium is obtained very efficiently. And, furthermore, only electrical power is consumed. There is no need for shipping, storing, and discarding chemicals.

#### Examples

Various eluates containing uranyl salts, mineral acids, and metal or ammonium salts of the acids were employed as catholytes in the electrolytic process described above. Aqueous solutions of the corresponding metal or ammonium salts were employed as anolytes. The cells were constructed of polymethyl methacrylate (Plexiglas). The electrodes were platinum, although carbon and copper are quite satisfactory as cathodes. With nitrate anolytes graphite anodes show reasonable durability whereas lead anodes are satisfactory with sulfate anolytes and can replace the platinum. The cells were divided into anode and cathode compartments by means of either an anionic or a cationic permselective membrane (Amberplex A1 or C1) known to contain about 70% ion exchange resin in a matrix of polyethylene and known to have been made according to the process of U. S. patent applications Serial Nos. 202,577 and 205,413, now U. S. Patents Nos. 2,681,320 and 2,681,319 respectively, and the corresponding Canadian Patents Nos. 493,562 and 493,563 of June 9, 1953. The cationic membranes contained a cation exchange resin which was a sulfonated cross-linked copolymer of styrene and divinylbenzene while the anionic membranes contained an anion exchange resin made by aminating with a tertiary amine a cross-linked, chloromethylated copolymer of styrene and divinylbenzene.

During electrolysis the anolytes and catholytes were mechanically agitated. The direct current was passed until the formation of a precipitate appeared to be complete, after which the catholyte was filtered to remove the hydrated uranium oxide. The filtrate and the anolyte were analyzed.

In the results which are tabulated below the concentration of the acids and salts is expressed in normality (N), A. E., percent, represents the percent of ampere efficiency of the process, and the concentration of uranium (U) is expressed in grams per liter (g./l.). Anionic permselective membranes were employed in obtaining the data below, but essentially the same results are obtained through the use of a cationic membrane.

| Cathode Solution               |                               |                   |          |                 | Anode Solution                 |                       |                |
|--------------------------------|-------------------------------|-------------------|----------|-----------------|--------------------------------|-----------------------|----------------|
| Initial Salt                   | Initial Acid                  | Initial U (g./l.) | Final pH | Final U (g./l.) | Initial Salt                   | Final Acid            | A. E., Percent |
| 0.9 N $\text{KNO}_3$           | 0.15 N $\text{HNO}_3$         | 5                 | 11.4     | 0.04            | 0.9 N $\text{KNO}_3$           | 0.19 N $\text{KNO}_3$ | 90             |
| 0.9 N $\text{KNO}_3$           | 0.1 N $\text{HNO}_3$          | 5                 | 7.5      | 0.03            | 0.9 N $\text{KNO}_3$           | 0.19                  | 89             |
| 0.9 N $\text{NH}_4\text{Cl}$   | 0.1 N $\text{HCl}$            | 5                 | 6.7      | 0.0             | 0.9 N $\text{NH}_4\text{Cl}$   | 0.20                  | ca. 100        |
| 0.9 N $\text{Na}_2\text{SO}_4$ | 0.5 N $\text{H}_2\text{SO}_4$ | 5                 | 12.0     | 0.001           | 1.8 N $\text{Na}_2\text{SO}_4$ | 0.46                  | 90             |
| 0.9 N $\text{KNO}_3$           | 0.1 N $\text{HNO}_3$          | 15                | 4.8      | 0.00            | 0.9 N $\text{NaNO}_3$          | 0.28                  | 88             |

I claim:

1. A process for the isolation of uranium compounds, which comprises passing a direct electric current through an electrolytic cell comprising a cathode compartment having therein an acidic aqueous solution which is made up of (a) a mineral acid from the class consisting of hydrochloric acid, nitric acid and sulfuric acid and (b) an alkali metal salt of said mineral acid and (c) a uranyl salt of said mineral acid, and an anode compartment hav-

ing therein an acidic aqueous solution which is made up of an alkali metal salt of a mineral acid from the class consisting of hydrochloric acid, nitric acid and sulfuric acid, said cathode and anode compartments being separated by 5 a permselective membrane which contains an ion exchange resin, continuing the passage of current until the hydrated uranium oxide has precipitated and thereafter separating said precipitated uranium compound from said catholyte.

10. The process of claim 1 in which the permselective membrane contains an anion exchange resin.

3. The process of claim 1 in which the permselective membrane contains a cation exchange resin.

4. The process of claim 1 additionally including the 15 step of igniting the hydrated uranium oxide to  $\text{U}_3\text{O}_8$ .

5. A process for the isolation of uranium compounds, which comprises passing a direct electric current through an electrolytic cell comprising a cathode compartment having therein an acidic aqueous solution which is made up of uranyl nitrate, an alkali metal nitrate and nitric acid, and an anode compartment having therein an acidic aqueous solution which is made up of an alkali metal nitrate, said cathode and anode compartments being separated by a permselective membrane which contains an ion exchange resin, continuing the passage of current until the oxide hydrated uranium has precipitated, and thereafter separating said precipitated uranium compound from said catholyte.

6. The process of claim 5 in which the permselective 20 membrane contains an anion exchange resin.

7. The process of claim 5 in which the permselective membrane contains a cation exchange resin.

8. The process of claim 5 additionally including the 25 step of igniting the hydrated uranium oxide to  $\text{U}_3\text{O}_8$ .

9. A cyclic process for isolating a uranium compound which is adsorbed on a bed of particles of an anion exchange resin which comprises first eluting said adsorbed compound by passing an aqueous solution of a mineral acid from the class consisting of hydrochloric acid, nitric acid and sulfuric acid and an alkali metal salt of the mineral acid through said bed of resin, collecting the eluate which contains the uranium in the form of a uranyl salt of said acid; electrolyzing said eluate in the cathode compartment of an electrolytic cell which contains a cathode compartment and an anode compartment separated by a permselective membrane containing an ion exchange resin, said anode compartment containing an aqueous solution of an alkali metal salt of the mineral acid present in said eluate; continuing the electrolysis until an insoluble uranium compound has precipitated; removing said uranium precipitate and transferring the remaining solution to the anode compartment of an electrolytic cell which is divided into an anode compartment and a cathode compartment by means of a permselective membrane containing an ion exchange resin; removing the anolyte from said first electrolytic cell and

transferring it to a bed of particles of an anion exchange resin on which is adsorbed a uranium compound; and repeating the electrolysis operation and the distribution of the products of the electrolytic operation.

10. The process of claim 9 in which said aqueous solution of a mineral acid and alkali metal salt is a solution of nitric acid and sodium nitrate.

11. A process for: (a) recovering uranium in the form 75 of uranium oxide and hydroxide from an aqueous solu-

tion derived from the elution of uranium complexes adsorbed by ion-exchange resins, and (b) for simultaneously reconditioning the eluate for further use in such elutions, said process comprising placing in the cathode compartment of an electrolytic cell, formed from a suitable container having a cathode and an anode compartment separated from each other by an ion-exchange resin-imregnated permselective membrane, an aqueous solution of a mineral acid from the class consisting of nitric, hydrochloric and sulfuric acids together with an alkali metal salt of said mineral acid and a uranyl salt of said mineral acid, placing in the anode compartment of said cell an aqueous solution of an alkali metal salt of a mineral acid, passing direct current through said cell until an insoluble uranium compound has precipitated in the catholyte, and filtering off the uranium precipitate from the catholyte, whereby the filtrate is made usable as the anolyte in a repetition of said process on another sample of eluate and after serving as the anolyte may be used in eluting a bed of ion-exchange resins which contain adsorbed uranium complexes.

## References Cited in the file of this patent

## UNITED STATES PATENTS

|           |                |               |
|-----------|----------------|---------------|
| 1,448,036 | Pearson et al. | Mar. 13, 1923 |
| 2,581,863 | Kahn           | Jan. 8, 1952  |
| 2,733,200 | Kunin          | Jan. 31, 1956 |
| 2,733,202 | Boyer          | Jan. 31, 1956 |
| 2,739,934 | Kunin          | Mar. 27, 1956 |
| 2,743,222 | Clevenger      | Apr. 24, 1956 |
| 2,776,184 | Kamen          | Jan. 1, 1957  |
| 2,781,303 | Boyer et al.   | Feb. 12, 1957 |

## FOREIGN PATENTS

|         |               |               |
|---------|---------------|---------------|
| 626,882 | Great Britain | July 22, 1949 |
| 493,562 | Canada        | June 9, 1953  |
| 493,563 | Canada        | June 9, 1953  |
| 704,602 | Great Britain | Feb. 24, 1954 |

## OTHER REFERENCES

- 20 Analytical chemistry of the Manhattan Project, C. J. Rodden, 1st ed., McGraw-Hill Book Co., New York, 1950; Div. VIII, pages 523-525.